

1

2,873,235

## ELECTRODEPOSITION OF COPPER

Frank Passal, Detroit, Mich., assignor to Metal & Thermite Corporation, Woodbridge Township, N. J., a corporation of New Jersey

No Drawing. Application June 19, 1957  
Serial No. 666,784

9 Claims. (Cl. 204—52)

This invention relates to electroplating of copper and more particularly to the electrodeposition of bright copper plates.

Electrodeposited copper is widely used as a decorative finish and also as an undercoat for subsequent electro-deposits such as nickel and/or chromium. Electroplating baths acceptable to industry are desirably economic, stable, easy to maintain, and should have good plating characteristics. Alkaline-cyanide type baths are widely used because of their relatively high plating speeds, excellent throwing power, and ease of maintenance. Alkaline-cyanide electroplating baths and processes are described in "Modern Electroplating," edited by A. G. Gray, pages 194-225 (1953).

I have now discovered a process for plating bright electrolytic copper from alkaline-cyanide baths containing novel additives.

It is an object of this invention to provide an efficient and economical process for electrodepositing bright and smooth copper deposits.

Another object of the invention is to provide bath compositions of the alkaline-cyanide type from which bright copper plate is electrodeposited.

Still another object of the invention is to provide compositions of matter which, when dissolved in water, yield alkaline-cyanide electrolytes suitable for the electrodeposition of bright copper electrodeposits.

Generally speaking, the invention contemplates electrodepositing copper from an alkaline-cyanide copper plating bath containing a small but effective amount of a compound having the general formula



(herein referred to as a tellurium dithiocarbamate), wherein R and R' may be the same or different and are selected from the class consisting of hydrogen and alkyl hydrocarbon groups having up to 6 carbon atoms in the group. R and R' within the scope of the invention include hydrogen and alkyl groups, such as methyl, ethyl, propyl, butyl, amyl and hexyl, and the branched as well as the straight chain groups. The R and R' groups may be replaced with a single alkyl cyclic compound, which may be viewed as a joinder of the R and R' groups and include compounds having a total of 5 to 7 carbon atoms in the chain. Tellurium diethyldithiocarbamate is the preferred additive.

Between about 0.001 g./l. (grams per liter) and 0.015 g./l., and preferably between about 0.006 g./l. and about 0.01 g./l. of the tellurium dithiocarbamate is included in the alkaline-cyanide copper plating baths.

Conventional alkaline-cyanide baths and process con-

2

ditions for electrodeposition are utilized in the present invention. Typical baths and process are illustrated in the table below:

|    |                                       | Range          |
|----|---------------------------------------|----------------|
| 5  | CuCN                                  | g./l. 30-90    |
|    | KCN                                   | g./l. 49-145   |
|    | K <sub>2</sub> CO <sub>3</sub>        | g./l. 0-112    |
|    | KOH                                   | g./l. 7.5-37.5 |
| 10 | KCN (free—adjusted to and maintained) | g./l. 5.6-11.2 |
|    | pH                                    | 13-13.8        |
|    | Temp.                                 | °F. 130-180    |
|    | Cathode C. D.                         | a. s. f. 10-50 |
|    | Anode C. D.                           | a. s. f. 10-20 |

15 The above table specifies baths and process limitations commercially preferred, and it is understood that the compositions and conditions may be varied somewhat, and that in certain cases it may be desirable to vary these limitations. The potassium salts noted in the table, 20 which are preferred, may be partially or completely replaced by sodium salts.

25 The copper electrodeposits obtained from baths utilizing tellurium dithiocarbamate additions are substantially mirror bright. The electrodeposits prepared from the tellurium dithiocarbamate-containing baths may be obtained in an even brighter condition by utilizing auxiliary or cooperating brightening additives in conjunction with the primary tellurium dithiocarbamate. Such auxiliary additives include relatively small amounts of salts of

30 lead, bismuth, antimony, or zinc, e. g., lead acetate, bismuth citrate, potassium antimony tartrate, zinc chloride, zinc sulfate, etc.

The alkaline-cyanide baths utilized should preferably contain a compound selected from the class consisting 35 of the alkali metal tartrates, citrates, gluconates, and saccharates.

Conventional wetting agents of the kind generally used in alkaline-cyanide copper electroplating baths are preferably incorporated in the baths. These include quaternary 40 amine wetting agents such as C-decylbetalaine and the ammonium hydroxide derivatives such as trimethylbenzylammonium chloride. We prefer novel and stable wetting agents of the following general structure:



(an alkyl  $\beta$ -amino propionate) or  $\text{RN}(\text{CH}_2\text{CH}_2\text{COONa})_2$  (an alkyl  $\beta$ -amino dipropionate). The above compounds, marketed under the trade name Deriphats, are used in concentrations of 0.01 to 0.1 gram per liter. They are 50 stable in the electrolyte and even impart some brightening action. A compound of this class which has been successfully used is the sodium salt of a coconut alcohol derivative of  $\beta$ -amino propionate designated as Deriphat 151.

55 Best results are usually achieved when utilizing in the electrodeposition process a method of preventing the thin film immediately adjacent to the cathode from becoming depleted in metal (copper) ion content. This is conventionally accomplished by agitation e. g., solution pumping, cathode movement, air agitation, etc., or by diffusion effects, e. g., current interruption, periodic current reversal etc., or by combinations thereof. Superior results have been achieved by utilizing current interruption in conjunction with cathode movement.

60 The following examples are illustrative of the present process and it will be understood that the invention is not limited thereto.

## 3

## Example No. 1

|                                                |                                 |
|------------------------------------------------|---------------------------------|
| CuCN                                           | 45 g./l.                        |
| KCN                                            | 72.5 g./l.                      |
| KOH                                            | 15 g./l.                        |
| KC <sub>6</sub> H <sub>11</sub> O <sub>7</sub> | 45 g./l. (potassium gluconate). |
| Tellurium diethyl dithiocarbamate)             | 0.008 g./l.                     |
| Deriphat 151                                   | 0.05 g./l.                      |

## Example No. 2

|                                                             |                                  |
|-------------------------------------------------------------|----------------------------------|
| CuCN                                                        | 45 g./l.                         |
| KCN                                                         | 72.5 g./l.                       |
| KOH                                                         | 15 g./l.                         |
| K <sub>2</sub> C <sub>6</sub> H <sub>8</sub> O <sub>8</sub> | 45 g./l. (potassium saccharate). |
| Tellurium dimethyl dithiocarbamate                          | 0.008 g./l.                      |
| Deriphat 151                                                | 0.05 g./l.                       |

## Example No. 3

|                                                                                   |                                  |
|-----------------------------------------------------------------------------------|----------------------------------|
| CuCN                                                                              | 45 g./l.                         |
| KCN                                                                               | 72.5 g./l.                       |
| KOH                                                                               | 15 g./l.                         |
| K <sub>2</sub> C <sub>6</sub> H <sub>8</sub> O <sub>8</sub>                       | 45 g./l. (potassium saccharate). |
| Tellurium diethyl dithiocarbamate                                                 | 0.008 g./l.                      |
| Pb(C <sub>2</sub> H <sub>3</sub> O <sub>2</sub> ) <sub>2</sub> ·3H <sub>2</sub> O | 0.0037 g./l. (.002 g./l. Pb).    |
| Deriphat 151                                                                      | 0.05 g./l.                       |

The bright copper electrodeposits obtained from the tellurium dithiocarbamate containing alkaline-cyanide baths of the present invention are obtained on such conventional basis metals as iron, steel, nickel, zinc, lead, copper, etc., and alloys thereof. On certain basis metals such as iron or steel and zinc-base die-castings the basis metal is first given an initial thin flash of copper from a low efficiency cyanide copper bath.

As many embodiments of this invention may be made without departing from the spirit and scope thereof, it is to be understood that the invention includes all such modifications and variations as come within the scope of the appended claims.

I claim:

1. An alkaline-cyanide bath for bright copper plating comprising copper cyanide and, as a brightening agent more than 0.001 g./l. of at least one tellurium dithiocarbamate having the general formula:



wherein R and R' are selected from the class consisting of hydrogen and alkyl groups having up to six carbon atoms.

2. A bath solution according to claim 1 in which the tellurium dithiocarbamate is tellurium diethyldithiocarbamate.

3. A bath solution according to claim 1 where the tellurium dithiocarbamate is present in amounts of between about 0.001 g./l. and 0.015 g./l.

10 4. A bath solution according to claim 2 where the tellurium diethyldithiocarbamate is present in amounts between about 0.006 g./l. and 0.01 g./l.

5. A bath solution according to claim 1 which also contains at least one secondary brightening agent selected from the class consisting of the salts of lead, bismuth, antimony and zinc.

6. In the process of electrodepositing copper from an alkaline-cyanide copper bath comprising copper cyanide, the improvement which comprises incorporating in said bath more than 0.001 g./l. of a tellurium dithiocarbamate having the general formula:



wherein R and R' are selected from the class consisting of hydrogen and alkyl groups having up to six carbon atoms.

7. The process as claimed in claim 6 in which between about 0.006 g./l. and 0.01 g./l. of tellurium diethyldithiocarbamate is incorporated in the bath.

8. A bath solution according to claim 1 which also contains an alkali metal gluconate.

9. A bath solution according to claim 1 which also contains an alkali metal saccharate.

## References Cited in the file of this patent

## UNITED STATES PATENTS

40 2,689,216 Nevers et al. Sept. 14, 1954

## OTHER REFERENCES

Meyer et al.: Transactions Electrochem. Soc., vol. 73 (1938), pages 377-413.

Serial No. 351,241, Weiner (A. P. C.), published May 18, 1943.

50